

## UNITED STATES PATENT OFFICE

1,931,072

## ASPHALTIC EMULSION

Donald McK. Hepburn, Philadelphia, Pa., assignor to Amiesite Asphalt Company of America, Camden, N. J., a corporation of New Jersey

No Drawing. Application September 14, 1929  
Serial No. 392,735

5 Claims. (Cl. 134—1)

This invention relates to aqueous emulsions of the asphalts, such as are used for binding the mineral aggregate of a road paving and more particularly to the production of an emulsion or dispersion of asphalt in water which has a substantially larger asphaltic content than those emulsions which have heretofore been made and consequently has a substantially smaller quantity of the menstruum water.

10 The object of this invention is to produce a dispersion of asphalt in a relatively small quantity of water or in a proportion of water substantially smaller than that heretofore used in making asphaltic emulsions for the binders of aggregate and to obtain a richer emulsion of asphalt and at the same time to so treat the asphalt that when it is precipitated from the menstruum or when the water is evaporated therefrom, as a result of coating objects therewith, the viscosity, 15 toughness, cohesiveness, adhesiveness, water resistance of the asphalt are all substantially increased and the penetration, as measured by a Dow penetrometer, is substantially decreased.

A further object of this invention is to produce an asphaltic cement for aggregate or for coating other objects than stone aggregate, which may be applied to and which will firmly adhere to the object whether the object be dry or wet at the time of the application of the emulsion thereto.

20 A further object of this invention is to produce a slow setting asphaltic cement for aggregate of such a character that mineral aggregate may be coated therewith at a plant remote from the road building operation and shipped thereto, or may be stored until ready for use, without having the coated pieces of aggregate firmly agglomerate in transit or storage.

A further object of this invention is to produce an asphaltic emulsion which will form on the stone a thicker coating than that obtainable from the use of emulsions of asphalts heretofore used for the purpose.

A further object of this invention is to form an aqueous dispersion of asphalt in water without making necessary the use of an oily volatile liquefier.

The preferred manner of making the binding and coating material constituting the present invention consists in dissolving substantially 25 parts, by weight, of soap in substantially 78 parts by weight of warm water. To the soapy water thus formed is slowly added, with vigorous agitation, about 20 parts, by weight, of a low grade fuel oil or a crude oil having an asphaltic base,

to produce a dispersion of the oil, in the warm soapy water.

The oil that is preferred for the practice of this invention is low grade fuel oil, by which is meant an oil that is low in cost and comparatively low in heat units, but having a substantial asphaltic content (preferably about 10%), because such oils contribute to the reduction in the cost of the material produced; because they soften and make workable the asphalt; and because they enable one to use a relatively tough asphalt for the production of an emulsion. Unless specifically stated, however, the invention is not to be construed as limited to the use of a low grade fuel oil, because other oils may be used in lieu of fuel oil with considerable success.

The low grade fuel oil which is preferably used should have an asphaltic content of substantially 10% or more as measured by precipitation with 86° naphtha; should contain a rather high percentage of unsaturated hydrocarbons, showing an iodine value of 40 or more; and should have a specific gravity of from .95 to .98. For convenience herein, the term "emulsive" oil is used to include fuel oil, crude oil, or any of the relatively involatile heavy oils usually used as liquefiers or fluxes for the asphalts in paving mixtures, and "fuel oil" is herein used to define the common oils on the market and used for burning in plants or residences for heating purposes; among which are those oils known in the trade as "Bunker C Gulf oil" and "Sun Bunker oil".

After the emulsion or emulsive oil has been made in the soapy water, a relatively small quantity of a metallic salt of a fatty acid is added to the emulsion and distributed or dispersed therein with thorough agitation or stirring. The salt preferably used in the process is aluminum oleate, but aluminum stearate or calcium oleate or stearate, or the stearates or oleates of zinc, iron and similar metals similarly increase the ductility of the asphalt and lower the penetration index or number thereof, and hence any of these metallic salts of the fatty acids may be used successfully in the practice of this process, and are fully within the scope and purview of this invention.

The amount of oleate or stearate so added to the emulsion is small, preferably from 1 to 2 parts by weight.

The salt of the fatty acid having been uniformly distributed throughout the emulsion, asphalt, preferably heated, is now slowly added thereto, with agitation, until substantially 296 parts, by weight, have been added thereto and distributed uniformly throughout the mixture. 110

During the mixing of the asphalt with the emulsion and the dispersing of the asphalt therein, the materials are thoroughly stirred or otherwise agitated and the best results will be obtained if the mixture is kept heated. The temperature at which the mixture is maintained is not very important so long as it is below the boiling point of water, for it is undesirable to substantially reduce the water which constitutes the menstruum of the emulsion prior to the application of the emulsion to the aggregate.

Nor is it necessary to the success of this process that the oleate or that the fuel oil be added at any definite stage of the process so long as they are reduced to a dispersion in water at the time of the final mixing operation.

Thus the oleate may first be mixed with the fuel oil or with the asphalt, or the fuel oil may first be mixed with the asphalt prior to the introduction of the asphalt into the soapy water. But for satisfactory results the order of steps first above given are preferred.

By thoroughly stirring or otherwise agitating the oil, asphalt and oleate in the presence of soapy water an emulsion will be formed, and once formed it is fairly stable. If during transportation or storage, the emulsion should tend to separate or stratify, a simple rolling of the barrel or a stirring of the contents thereof will suffice to re-distribute and disperse the suspended matter throughout the water. Fuel oil, such as has been above described, is preferred because such heavy oils are of more uniform consistency and composition than crude oils, which generally contain more or less of the lighter volatile oils, and because they contain substantially no volatile oils. When crude oil is used as a substitute for the fuel oil in the practice of this invention, the proportion of the ingredients used in making the binding composition and the temperatures to which the ingredients are heated should be varied to correspond with the amount of volatile lighter oils contained in the crude oil. Moreover, crude oils vary very much in composition and in consistency and each crude oil should be carefully sampled and tested to determine the asphaltic content and the amount of lighter oils contained therein in order that the process may be successfully performed.

The action of the salt of the fatty acid in the presence of the asphalt contained in the mixture appears to be a chemical one, for after the emulsion has been applied to the aggregate and the water has evaporated therefrom, the asphalt is tougher, and has a lower penetration than it had when it was added to the emulsion. The tenacity with which the coating adheres to the aggregate and with which the coated pieces of aggregate cohere to each other, is substantially increased, and a thicker coating of asphalt is formed on the surface of the aggregate than that obtainable from any other emulsion of asphalt of which the applicant herein has any knowledge. Briefly, the process consists in thoroughly agitating asphalt in the presence of an emulsive oil, and a small quantity of the salt of a fatty acid, in warm soapy water, the combined weight of the oil and the as-

phalt being about 4.25 times the weight of the water in which said asphalt and oil are dispersed.

Having thus described my invention, what I claim and desire to protect by Letters Patent of the United States is:

1. A bituminous composition adapted to and ready for application without heating to an unheated aggregate comprising a dispersion in soapy water of asphalt substantially 296 parts, an involatile heavy emulsified oil substantially 20 parts, a salt of a fatty acid having a greater affinity for oils than for water, from 1 to 4 parts and water soluble soap substantially 9 parts, the proportions given being by weight.

2. A bituminous composition adapted to and ready for application without heating to unheated aggregate comprising a dispersion in water of asphalt substantially 296 parts, an involatile bituminous fuel oil substantially 20 parts, a salt of a fatty acid having a greater affinity for oils than for water, substantially 1 part and a water soluble soap substantially 9 parts.

3. A bituminous composition adapted to be directly applied, without heating, to an unheated mineral aggregate and comprising water, soap and involatile fuel oil containing substantially 10% of asphalt, a salt of a fatty acid, said salt having a greater affinity for oils than for water, and bitumen, the above ingredients being in substantially the following proportions by weight,

|                           | Parts  |
|---------------------------|--------|
| Water                     | 78     |
| Soap                      | 9      |
| Involatile fuel oil       | 20     |
| Said salt of a fatty acid | 1 to 2 |
| Bitumen                   | 296    |

4. The method of making a bituminous cement, which consists in dissolving water-soluble soap in warm water, slowly adding thereto fuel oil with vigorous agitation to form a dispersion of the oil in the water, mixing therewith a water-insoluble, water-indispersible metallic salt of a fatty acid, and slowly adding to the mixture under continuous vigorous agitation, melted bitumen, the proportions of the ingredients by weight being substantially,

|                                    | Parts  |
|------------------------------------|--------|
| Soap                               | 9      |
| Water                              | 78     |
| Fuel oil                           | 20     |
| Said metallic salt of a fatty acid | 1 to 2 |
| Bitumen                            | 296    |

5. The method of making a bituminous cement, which consists in dispersing a fuel oil (substantially 20 parts), in water (substantially 78 parts), containing a water-soluble soap (substantially 9 parts), adding thereto a small quantity (from 1 to 2 parts) of a metallic salt of a fatty acid, said salt having a greater affinity for oils than for water and slowly adding to the mixture under vigorous agitation, melted bitumen (substantially 296 parts) and continuing the agitation until the mass is homogeneous, the above proportions being by weight.

DONALD MCK. HEPBURN.